

# UNITED STATES PATENT OFFICE.

SAMUEL E. BRICK, OF SALINA, KANSAS; LILLIAN B. BRICK EXECUTRIX OF SAID  
SAMUEL E. BRICK, DECEASED.

## BOOKBINDING-GUM.

1,389,574.

Specification of Letters Patent. Patented Sept. 6, 1921.

No Drawing.

Application filed February 1, 1919. Serial No. 274,554.

*To all whom it may concern:*

Be it known that I, SAMUEL E. BRICK, a citizen of the United States, residing at Salina, in the county of Saline and State of Kansas, have invented certain new and useful Improvements in a Bookbinding-Gum, of which the following is a specification.

This invention relates to adhesives and more particularly to an improved tabbing 10 and book binding gum.

The primary object of this invention is to provide an improved gum having advantages over the tabbing gum described in my co-pending application, Serial #237,771, 15 filed June 1, 1918.

The ingredients, are:

One and one-quarter pounds of celluloid,  
One gallon of acetone

One gallon of unsmoked gum rubber.

20 The quantities referred to above will indicate the proportions which may be used to the best advantage although it will be understood that these proportions may be changed to some degree, for securing the desired re-

25 sults.

In preparing the compound, I proceed as follows:

The raw unsmoked gum rubber is placed 30 in an agitator or mixer and is cut in a quantity of benzol until a very thick paste results. The mixer or agitator should be kept in actuation until a paste about as thick as glucose has been formed. The unsmoked rubber gum is more desirable than the 35 smoked rubber for the reason that it is stronger and is of a lighter color, and a coloring may thereby be added for the purpose of coloring the compound to a shade lighter than would be obtainable with the 40 smoked rubber. It should be borne in mind, however, that the smoked rubber may be employed if for any reason it is found desirable although if the compound is colored after being prepared, only the darker shades 45 can be obtained. Tetrachlorid of carbon may be used in place of benzol if desired and it will be found that this cuts the rubber gum sufficiently to provide the paste but it has the disadvantage of evaporating more 50 rapidly than benzol and if the container is left open while the mixture is being made into the paste, care must be used to prevent

the paste becoming too thick because of the rapid evaporation of the tetrachlorid of carbon. The latter, however, has the advantage 55 of having a less objectionable odor.

The celluloid is then cut in the acetone by placing the celluloid and acetone in a suitable mixer or agitator whereupon the latter is kept in operation until the mixture 60 has the proper consistency so that the gum paste and the celluloid mixture are combined and thoroughly mixed. The celluloid most desirable and from which the best results are secured is the so-called sheet celluloid such as is commonly used by automobile top manufacturers. The waste scraps of sheet celluloid are thereby rendered valuable and while I have been using these scraps to advantage, it should be understood that 70 any other celluloid may be employed in making the compound so long as it is soluble in acetone and contains no mineral or oxid.

After the mixture has been thoroughly agitated it can be colored any shade desired. 75

While it has been found desirable to mix equal portions of the celluloid mixture with the rubber mixture, it should be understood that any changes in the proportion might be 80 made if a stiff or flexible backing is desired when the compound is used for tabbing and bookbinding. If the proportions are changed so that four-fifths of the celluloid mixture is added to one-fifth of the rubber 85 mixture the result will be a very stiff backing. If four-fifths of the rubber mixture is added to one-fifth of the celluloid mixture it will be found that the result is a very flexible tabbing and of course, these proportions 90 may be varied so that the desired flexibility may be obtained. It will be found that these changes in the proportions will not interfere with the drying and lasting qualities 95 of the compound. It should be also pointed out that the celluloid may be cut in both the acetone and the tetrachlorid of carbon by cutting the celluloid with one-half the quantity of acetone and then thinning the mixture with tetrachlorid of carbon. 100

Inasmuch as the compound is flexible, easily dried and may be applied with a brush and is always used cold, it will be readily understood that it is especially adapted for

tabbing and bookbinding. It needs no heating and will dry very quickly when applied and also possesses an attractive gloss which the compound described in my pending case above referred to does not possess.

Having thus fully described my invention what I claim as new and desire to secure by Letters Patent, is:—

A composition consisting of a solution of

celluloid and gum rubber in a mixture of 10 benzol, acetone and carbon tetrachlorid.

In testimony whereof I affix my signature in presence of two witnesses.

SAMUEL E. BRICK.

Witnesses:

O. H. FORREST,  
W. B. SMITH.